

June 8, 1937.

G. M. CROFT ET AL

2,083,433

METHOD OF TREATING METALS

Filed Oct. 11, 1934

4 Sheets-Sheet 1



Inventors:

GEORGE M. CROFT and  
JOHN A. HUNTER.

by:

Keena & Rucker  
Their Attorneys

June 8, 1937.

G. M. CROFT ET AL

2,083,433

METHOD OF TREATING METALS

Filed Oct. 11, 1934

4 Sheets-Sheet 2



*Inventors:*

GEORGE M. CROFT and  
JOHN A. HUNTER.

by: *Usina & Hauber*  
Their Attorneys.

June 8, 1937.

G. M. CROFT ET AL

2,083,433

METHOD OF TREATING METALS

Filed Oct. 11, 1934

4 Sheets-Sheet 3

*Fig. 4.*



*Inventors:*

GEORGE M. CROFT and  
JOHN A. HUNTER.

*by:*

*Uenia & Rumber*  
their Attorneys.

June 8, 1937.

G. M. CROFT ET AL.

2,083,433

## METHOD OF TREATING METALS

Filed Oct. 11, 1934

4 Sheets-Sheet 4

Fig. 5.



Fig. 6.



Fig. 7.



## *Inventors:*

GEORGE M. CROFT and  
JOHN A. HUNTER.

By:

Usina & Rauber  
their Attorneys.

## UNITED STATES PATENT OFFICE

2,083,433

## METHOD OF TREATING METALS

George M. Croft, Dormont, and John A. Hunter,  
Ben Avon, Pa., assignors to American Sheet  
and Tin Plate Company, a corporation of New  
Jersey

Application October 11, 1934, Serial No. 747,946

1 Claim. (Cl. 148—16)

This invention relates to a novel method of treating metals, and more particularly to the deoxidizing and bright annealing thereof.

In the manufacture of metals, and particularly highly finished sheet metals such as are intended for subsequent use as automobile bodies, commercial tin plate and the like, it is highly desirable to bright anneal or deoxidize the same.

It has been the practice in the past to deoxidize or reduce hot mill scale and other superficial surface oxides and bright anneal (to prevent reoccurrence on the surface of the highly finished sheet metal of oxides) by introducing hydrocarbon-bearing gases into a container in which the metal is disposed. The gas is usually either natural, coke-oven, coal or producer gas, and even the heavier hydrocarbons (such as propane and butane) in either a gaseous or liquid state.

20 These gases contain free oxygen and moisture and vary widely in composition. Due to this, they are readily broken down and invariably result in carbon or soot being deposited, in addition to which the oxygen and water causes blued, 25 or otherwise discolored, metal. These conditions are, of course, highly objectionable but had to be contended with as the annealing, or softening, of the metal is necessary. The complete deoxidation (reduction of oxides etc.) and bright annealing of metals (prevention of reoccurrence of oxides, etc.) has heretofore been impossible if raw hydrocarbon gases are used.

It is one of the objects of the invention to provide a novel method of treating metals which will effect the complete elimination of surface defects heretofore encountered in annealing operations.

Other objects will be apparent after referring to the drawings, in which:

40 Figure 1 is a schematic layout.

Figure 2 is a plan of a part of the apparatus.

Figure 3 is a view on the line III—III of Figure 2.

45 Figure 4 is a view on the line IV—IV of Figure 2.

Figure 5 is an end elevation of the part of the apparatus shown in Figures 2, 3, and 4.

50 Figures 6 and 7 are enlarged fragmentary details.

The gas reforming apparatus preferably used in carrying out the method of the invention comprises, in part a box or furnace A which is rectangular in shape, having ends 1, sides 2, bottom 3, and top 4, all of suitable steel plate,

welded or bolted together. The box or furnace A is lined with a suitable insulator brick 5 and mounted on supporting legs 6. A lifting lug 8 is attached to each corner of the box 4 to permit its easy transportation as a unit by means of 5 a crane (not shown).

Within the insulated box A are vertical tubes 9 connected in series by tubes 10. These tubes 9, and connecting tubes 10, are of a heat resisting alloy such as chromium or chromium-nickel bearing steel which is capable of withstanding the high temperatures to which they are subjected. The number of vertical and connecting tubes may vary, depending on the amount of hydrocarbon gas that is to be forced therethrough, 15 as well as the temperatures to which the gas is exposed. The ends of the tubes 9 extend through the top 4 and bottom 3 of the box A and are normally closed, as by caps 11. These tubes 9 are vertically suspended by means of bolted support- 20 clamps 12, which encircle them at the top 4 of the box A. The entire length of the tubes 9 and 10, with the exception of the first tube, which is indicated at 9a, may be filled with any substance 13 such as crushed brick, refractory, 25 or any such medium whose bond will not deteriorate and which will be capable of withstanding high temperatures and yet offer a maximum contact surface for the gases. It has been found from experiment that any first quality fire brick that will pass through a 1½" 30 screen is the most suitable medium due to the fact that it efficiently permits the transmittal of heat to the gas to be reformed, and at the same time is neutral with respect to any reaction 35 with steam which is admitted in the process.

The inactiveness of the refractory is also desirable in that it will allow the introduction of an excess amount of steam which is good insurance against plugging up of the box A by carbon that might precipitate from the gas during the reforming process. However, any heat resisting metal which will give maximum heating area and stand up as long as refractory material will give equal results. If the volume of gas to be treated is exceedingly great this refractory may be dispensed with and the tubes used in an empty condition.

The tubes 9 and 10 are heated by gas burners 14 disposed as shown (Figures 3 and 4) through the ends 1 of the box A. The heat input of the burners 14 is automatically, or manually, controlled by a pyrometer 15 which is disposed in the exit tube which is indicated at 9b. The waste gas,

or products of combustion, escape from the box A through vents 16 disposed on the ends and sides 1 and 2 adjacent the roof of the furnace.

The raw hydrocarbon bearing gas is introduced 5 into the box A through an inlet pipe 17. However, before it reaches the first tube 9<sup>a</sup> within the box it is caused to mix with an excess of steam which is injected through a pipe 18. The position of this steam inlet with relation to the gas burners 10 14 is best shown in Figures 5 and 6, and is slotted as at 18<sup>a</sup> to insure a homogeneous mixture of gas and steam.

The mixture of raw hydrocarbon bearing gas and excess steam is thus exposed to high heat 15 (about 1800 degrees-1900 degrees F.) as it travels through the tubes 9 and 10. This causes the reformation or breaking down of the basic constituents of the gas and producing principally hydrogen (H<sub>2</sub>) and carbon monoxide (CO) in varying 20 but controllable amounts.

The amounts of these reformed gases and the minute presence or total absence of oxidizing 25 mediums depend on the temperature to which the hydrocarbon gases are subjected and the ultimate use of the gas as hereinafter described in detail.

At this stage of the process carbon in the form 30 of soot may be precipitated out of the gas, but the carbon in the gas reacts with the excess steam. Any free oxygen is taken up by the new gaseous mixture and excess steam plus water vapor in the raw gas may precipitate in the last or exit tube 9<sup>b</sup> to be suitably and periodically drawn off by a collecting bulb and shut-off valve 35 19. While such a condition is exceptional it is, however, possible and therefore is anticipated.

Following the heating and breaking down of the hydrocarbon gas mixture within the box A or reforming furnace the reformed gas is conducted through an exit pipe 20 to a cooler B. This cooler B is for the purpose of condensing and removing any water vapor and excess steam that may still be retained by the gas, and is standard equipment such as is ordinarily used with air 40 compressors; utilizing ordinary mill water as a cooling medium. In the event that the mill water temperature runs between 70 degrees-100 degrees F., especially during the summer season, it has been found desirable to pass the gas coming from 45 this cooler through any standard refrigerating machine which is adjusted to chill the gas preferably to 35 degrees-40 degrees F. Suitable drains are provided on both types of coolers for draining off the condensed water vapor thus extracted from the gases as chilled.

At this point it has been found that the chilled reformed gases contain principally hydrogen, carbon monoxide and some methane together with small amounts of water and carbon dioxide. A 50 typical analysis might for example indicate: 50-60 per cent hydrogen (H<sub>2</sub>), 35-40 per cent carbon monoxide (CO) and remainder being methane (CH<sub>4</sub>); water vapor and steam (H<sub>2</sub>O) and carbon dioxide (CO<sub>2</sub>).

If this gas is to be used in the deoxidizing or reducing of oxides on sheet metal (such as hot-mill scale and the like) the presence of these small amounts of water vapor and carbon dioxide have not been found to work a hardship at the relatively high temperatures (1200 degrees F.-1500 degrees F.) which may be used in the deoxidizing treatment. However, if the gas is to be used in the presence of highly finished sheet, or strip (such as metals cold reduced on four-high cold reduction mills or the like), it must be further treated 75

so as to remove all gases except hydrogen, carbon monoxide and methane. To cause the removal of any water vapor, carbon dioxide, or any oxidizing media, the cooled reformed gases are again passed through the box or furnace A previously described. For this purpose a plurality of vertical tubes 21 and connecting pipes 22 are provided and connected in series in the same manner as tubes 9 and pipes 10.

These reheating tubes 21 are made of a suitable 10 alloy and contain charcoal 23 or a like substance capable of extracting from the reformed gases practically all of the water vapor and reducing 15 carbon dioxide to carbon monoxide which may still exist. This gas which is further "purified" 20 by its passage through the charcoal-containing tubes may well be used not only for the bright annealing of highly finished or surfaced sheet metal but also for deoxidizing, in which event a substantial improvement of product is obtained 25 over the otherwise unpurified gas. The gas is passed through these reheating tubes 21 and connecting tubes 22 from the cooler B by means of feed-pipes 24.

Following the exit of the reformed and purified 30 gas from the cooler B and the tubes 21, it is led through pipes 25 to a manifold 26, from where it is distributed to a plurality of annealing boxes 27 which are schematically shown in Figure 1. These annealing boxes 27 are of the conventional type comprising a base 28 and cover 29 of cast steel, or iron. The pile of metal, such as sheets 30 or coils 31, are placed on the base 28, the cover 29 placed thereover and a sand seal 32 maintained therebetween to prevent the entrance of air. A plurality of tubes 33 lead from the manifold 26, under the covers 29 and through the sand seals 32; thus introducing the reformed gas into the presence of the metal to be heated. The use of the reformed and purified gas is favored as it bears not only further purification but is in a preheated condition which shortens the desired heat cycle of the annealing boxes 27. The tubes 33, which lead from the manifold 26 under the covers 29 and through the sand seals 32, are provided with suitable quick-detachable connections, as at 33<sup>a</sup>.

If the metal is free from any metallic surface defects such as scale, pickle stains, or any degree of oxidation, the treatment confines itself to bright annealing. Bright annealing as accomplished by the use of the improved gas mixture is carried out at a relatively low temperature (950 to 1200° F.), the presence of the gas being only for the purpose of maintaining the bright, un-oxidized surface and preventing the reoccurrence 55 of oxides. The heat to which the sheets are subjected is, of course, for the purpose of annealing. The reformed gas should contain little or no carbon dioxide, oxygen or water vapor, and if such oxidizing media are present in very small 60 amounts they will be ineffectual due to the preponderant presence of hydrogen.

The purified and reformed gas, as it comes from the purifying and charcoal-containing tubes 21 contains approximately 61 per cent hydrogen (H<sub>2</sub>), approximately 35 per cent carbon monoxide (CO), the remainder of the gas containing principally methane (CH<sub>4</sub>).

It is to be understood by those skilled in the art that these percentages of hydrogen, carbon monoxide and methane will vary somewhat, depending on the type of raw gas or liquid hydrocarbons to be reformed and the time and temperatures to which they are subjected. Thus, for example, we have indicated that for bright an-

nealing of metal, the proportions given are quite satisfactory. The gas may, for example, result from the reformation of propane (C<sub>3</sub>H<sub>8</sub>) which is subjected to a breakdown temperature of about 5 1820° F. in the presence of excess steam in the box or furnace A, as previously described.

The same percentages of hydrogen and carbon monoxide as utilized in the bright anneal of metals just described can be applied equally well 10 in the deoxidizing treatment. This deoxidizing treatment is limited in this specific example to boxes or closed containers and involves relatively high heat treatments, such as, for example, 1200-1500° F.

15 The entire gas reforming equipment may be automatically controlled or operated by inserting specified size orifices (not shown) in the individual lines to each annealing box 27 and maintaining a constant pressure in the manifold 26 by means of a suitable gas pressure regulator. The flow to the boxes 27 will vary in accordance with the porosity of the sand seal 32 and the automatic temperature control will maintain a constant temperature in the furnace or box A. The 20 steam regulator may be set to deliver a constant pressure.

The deposits of carbon or soot on the metal are thereby eliminated, the objectionable oxides on such metal are completely reduced and no further discoloration or reoccurrence of oxides on the metals is possible through the more or less complete absence of oxygen and/or water vapor in our hydrogen-carbon monoxide mixture.

30 We find that, by the use of this high hydrogen and high carbon monoxide gas mixture produced from reformed hydrocarbons, the ultimate sur-

face of the sheet metal heated in the presence thereof is extremely well adapted to receive protective and decorative coatings such as lacquers, paints and lithographic mediums. This metal surface having been exposed to gas under heat 5 apparently takes a thinner and more uniform coating of various paints for protective or decorative purposes than metals whose surfaces have been cleaned by raw gases or acids.

We further find that such reformed gases 10 act on and remove oil from the surface of metals, such as sheet or strip metal, piled flat, or in coils, which have been previously subjected to a processing step which left a film of oil (lubricating or preservative) upon their surfaces. It has 15 heretofore been practically impossible to remove this oil film without causing discoloration, especially of sheet or strip metals as bright annealed.

While we have shown and described one specific embodiment of our invention, it will be understood that we do not wish to be limited exactly thereto, since various modifications may be made without departing from the scope of our invention, as defined in the following claim. 25

We claim:

A method of treating metals which includes heating the same and subjecting the heating metal to a broken down and reformed gas consisting of approximately 61 per cent of hydrogen, 30 35 per cent of carbon monoxide and the remainder methane, said gas being devoid of any influential oxidizing medium.

GEORGE M. CROFT. 35  
JOHN A. HUNTER.